

## [54] CONTINUOUS ELECTROWINNING CELL

[75] Inventor: Robert Clarence Emmett, Jr.,  
Dundee, Ill.[73] Assignee: Envirotech Corporation, Salt Lake  
City, Utah

[22] Filed: Feb. 20, 1973

[21] Appl. No.: 334,157

[52] U.S. Cl..... 204/281, 204/10, 204/216

[51] Int. Cl..... B01k 1/00, C22d 5/00, B23p 1/00

[58] Field of Search ..... 204/10, 225, 216, 208,  
204/281, 13

## [56] References Cited

## UNITED STATES PATENTS

|           |         |                     |         |
|-----------|---------|---------------------|---------|
| 1,251,302 | 12/1917 | Tainton.....        | 204/10  |
| 1,959,376 | 5/1934  | Lucas.....          | 204/10  |
| 2,805,986 | 9/1957  | Law .....           | 204/281 |
| 3,414,486 | 12/1968 | Nordblum et al..... | 204/10  |
| 3,419,901 | 12/1968 | Nordblum et al..... | 204/10  |

## FOREIGN PATENTS OR APPLICATIONS

178,994 4/1966 U.S.S.R..... 204/10

Primary Examiner—T. M. Tufariello

Attorney, Agent, or Firm—Robert R. Finch

## [57] ABSTRACT

An electrolytic cell is formed with a housing enclosing a flat-faced cathode and anode in closely spaced face-to-face relationship. The cathode comprises a plurality of small diameter cathode elements held in spaced-apart relationship by an insulating matrix. Each of the elements terminates in a small diameter tip. Metal deposits on the tips in dendritic form and is scraped therefrom. The anode face is porous and connections are provided for withdrawing gaseous products from the face as they are formed. Operation is continuous, recovered metal being flushed from the cell in spent electrolyte as the latter is displaced by fresh electrolyte.

12 Claims, 8 Drawing Figures



PATENTED JAN 14 1975

3,860,509

SHEET 1 OF 2



FIG. 1



FIG. 2

PATENTED JAN 14 1975

3,860,509

SHEET 2 OF 2



FIG. 3



FIG. 4



FIG. 5



FIG. 8



FIG. 6



FIG. 7

## CONTINUOUS ELECTROWINNING CELL

## BACKGROUND OF THE INVENTION

## 1. Field of the Invention

This invention relates to an apparatus and process for the continuous electrowinning of metal.

## 2. State of the Art

Electrowinning, a well-known process, utilizes an electric current to reduce an ionized metal for deposit as elemental metal on a cathode. The ionized metal is carried in an electrolyte usually yielded from an acid leach of a metal bearing ore or concentrate. A conventional electrowinning cell comprises a tank in which one or more sets of insoluble anodes and cathodes are immersed in an electrolyte. When a current passes through the electrolyte between the electrodes, metal is deposited on the cathode.

As currently practiced, electrowinning is a batch operation conducted in large tanks in which a plurality of cathodes and anodes are suspended. The anodes are usually chemically inert, typically, a lead alloy such as lead-antimony. The cathodes are usually thin starting sheets of the same metal as that which is to be recovered and are retained in the electrolyte for one to three weeks until a commercially usable quantity of metal builds on them.

Batch operations have several drawbacks. These include the need for a large amount of floorspace to achieve acceptable production rates and the fact that new starting cathodes must be supplied for each new batch.

Attempts have been made to improve on batch metallurgy. One proposal for doing so is the powder metallurgy technique in which very high current densities are employed under conditions such that the metal deposits on the cathode as a powder rather than a solid plate. In such form, the metal may often be scraped from the cathode while the latter is in place in the cell. Although powder metal is easy to harvest, it usually contains many occluded impurities and its granular characteristics, such as bulk density, are often unacceptable for use except with further purification.

## SUMMARY OF THE INVENTION

This invention provides improved ways and means for continuous electrowinning of metal in commercial acceptable form. The mechanism includes a cathode of novel construction on which metal is deposited as small dense particles. Means are provided for continuously removing deposited metal while electrolysis continues.

The cathode is formed so that its exposed face comprises a plurality of small-area tips held in spaced-apart relationship by an insulating matrix. With this construction, each small-area tip functions as a separate cathode. The invention is predicated on the discovery that if the individual cathode tips have a small exposed area, metal will deposit thereon in a particular configuration and with such a fragile bond that it is subjected to easy harvesting without harming the tips. A harvesting means is provided to continuously remove deposited metal from the cathode tips, and means are also provided to remove the metal particles from the cell as they are harvested. A porous anode of special design is also provided to continuously withdraw gaseous products from the cell.

## BRIEF DESCRIPTION OF THE DRAWINGS

The present invention may be more readily understood and carried into effect by reference to the following description and appended drawings which are offered by way of illustration and not in limitation of the invention, the scope of which is defined by the appended claims and equivalents thereof rather than by any separate description.

## 10 In the drawings:

FIG. 1 is a side view of an electrolytic cell embodying the invention. For purposes of illustrating internal components, a portion of the cell wall is shown as partially cut away;

## 15 FIG. 2 is a plan view of the cell illustrated in FIG. 1 with portions of the wall cut away for purposes of revealing internal components. Additionally, electrolyte supply piping is also illustrated;

## 20 FIG. 3 is a pictorial view, partially cut away, of the cathode employed in the cell illustrated in FIGS. 1 and 2;

## 25 FIG. 4 is a sectional view taken in a plane passing through the line 4-4 of FIG. 3 and viewed in the direction of the arrows 4;

## 30 FIG. 5 is an enlarged detailed view of that part of the cathode encompassed within the line 5-5 of FIG. 4;

## 35 FIG. 6 is a pictorial view of an anode suitable for use in the cell illustrated in FIG. 1;

## 40 FIG. 7 is a sectional view taken in a plane passing through the line 7-7 of FIG. 6 and viewed in the direction of the arrows 7; and

## 45 FIG. 8 is a detailed view of a metal harvesting means adapted for use with the cell.

## DETAILED DISCLOSURE

The electrowinning cell illustrated in FIGS. 1 and 2 generally comprises a housing 12 in which are mounted a cathode 13 and an anode 14 in face-to-face relationship. The housing 12 may be sealed to facilitate capture of gaseous products of electrolysis and prevent escape of corrosive vapors. The inner wall of the housing is electrically insulated, preferably with a corrosion-resistant material.

45 The cathode 13 is designed so that metal of proper characteristics will be efficiently deposited thereon at a high rate and in a form susceptible to continuous removal without damage to the cathode or interruption of the process. As shown in FIGS. 3-5, the cathode 13 comprises a plurality of exposed electrically conductive tips 30, each of which functions as a separate cathodic element. The tips are the terminal ends of thin conductors 31, such as small-diameter wires, which are supported in spaced-apart relationship by a matrix of insulating material 32 held in an insulated holder 43 with only the tips 30 exposed. The other ends of the conductors 31 are all connected inside the holder to a common electrically conductive base 34. The exposed surface or face of the cathode 13 should be smooth so that deposits on the individual cathode tips do not physically stick to the insulating matrix 32 and none of the sidewalls of the individual cathodic elements 31 are exposed. Thus, the conductive cathode surface may be described as being a smooth surface formed from the free ends of a plurality of electrical conductors held in spaced-apart relationship by a matrix of non-conducting material.

50 The cathode tips 30 are sufficiently small that the metal deposits thereon in a configuration which exhib-  
55  
60  
65

65 The cathode tips 30 are sufficiently small that the metal deposits thereon in a configuration which exhib-

its a weak bond and extends outwardly from the cathode face, thereby enhancing removal by a light scraping action. As illustrated, the cathode tips are flat, round surfaces about 0.025–0.15 mm in diameter (area =  $0.0005\text{mm}^2$  to  $0.018\text{mm}^2$ ) and the edges of the tips are spaced 0.25–0.6 mm apart at the closest points. As shown in FIG. 5, metal deposits on the cathode tips 30 in the form of small outwardly extending clumps 41. The clump-tip bond is small and easily broken. The small tips are important because if the diameter of the tip surface is increased appreciably, two undesirable things occur: first, the bonding area increases so that deposited metal adheres more firmly and, second, the deposited metal tends to spread radially about the tip and takes a disc-like configuration that is difficult to remove and which will also contribute to undesirable bridging between tips. As noted, the spacing between adjacent tips is also important and should be in the range of 0.25 to 0.6 mm to insure that deposited metal does not form a bridge between adjacent tips.

One technique for fabricating a suitable cathode is to first fix segments of relatively large diameter stainless steel wire to a base strip to provide a comb-like component. A number of such strips are fixed together to form a brush-like cluster. The diameters of the wires are then decreased by known etching techniques and the cluster is encapsulated in a suitable insulating material such as a ceramic, glass or appropriate plastic. The insulating material should be corrosion-resistant and of sufficient strength that it does not flex or permit working loose of the conductors to the extent that greater cathode areas are exposed lest the character of the metal deposits change and they become difficult to remove.

It is not necessary that the conductors 31 be wires or that they be round. Suitable cathodes have been formed where the individual tips have a rectangular configuration, say 0.025–0.1 mm by 0.5–2.5 mm (area =  $0.0125\text{mm}^2$  to  $0.25\text{mm}^2$ ), and with spacing between adjacent tips ranging from 0.25–0.6 mm at the closest points. Again, the spacing is important to avoid bridging between adjacent tips.

Referring again to the illustrated cathode, one end of an insulated shaft 46 is rigidly fixed to and extends from the rear face of the cathode holder 43 to extend through the adjacent endwall of the housing 12 where it connects to a suitable drive 48 adapted to effect slow rotation of shaft 46 and the cathode holder 43. A conventional stuffing box 49 encircles the shaft where it exits the housing. An electrical conductor 51 (FIGS. 3 and 4) extends from the common base 34 through the insulated shaft 46 to terminate outside the housing at a contactor 51a adapted to be connected to a direct current source, not shown, but which typically supplies a potential of about 2–8 volts across the electrodes. If the cell contains more than one pair of electrodes, the DC source should be capable of supplying 2–8 volts across each pair.

The anode 14 (FIGS. 6–7) is designed to serve as the inlet for fresh electrolyte simultaneously with removal of gaseous electrolysis products. The anode includes a flat face plate 53 made from a perforated or otherwise porous material. For instance, the plate 53 may comprise two super-imposed layers of perforated titanium sheet which are coated with a metal or oxide capable of functioning as an inert anode whereby to promote oxygen release. When assembled in the housing, the

anode face plate 53 forms the conductive anode surface and is in closely spaced parallel relationship to the conductive cathode surface 13.

The face plate 53 fits over a hollow cylindrical holder 54 in which is fitted a solid divider 55 which divides the anode transversely into a front chamber or plenum 56, just back of the anode face plate, and a back chamber or plenum 57 adjacent the rear of the holder. The holder and the divider should be made from non-conductive, anodic-corrosion-proof material. An insulated shaft 58 is connected and extends rearward from the holder. A suitable conductor 67 extends through the shaft to connect the face plates 53 to the D.C. source. A plurality of short, electrically non-conductive conduits 59 extend through the divider 55, thence across the front chamber 56 and through the anode face plate 53 to thus provide communication between the rear chamber 57 through the face plate 53 into the interior of the housing 12. A bore 61 in the shaft forms 20 a conduit which connects the back chamber 57 to a source of electrolyte, all as more fully described hereinafter.

A second bore 63 extends longitudinally through the shaft 58 thence through the back chamber 57 and the 25 divider 55 to provide communication between the front chamber 56 and the exterior of the anode whereby enabling withdrawal of gas through the porous anode face 53. In some cases the withdrawal of gas may be facilitated by application of vacuum to the front chamber via conduit 63 in addition to the pressure differential created by introduction of electrolyte.

The electrolyte supply conduits 59 are sized and spaced on the anode face 53 to permit an adequate supply of fresh electrolyte into the housing 12 without unnecessary jetting that might result in premature removal of metal deposits from the face of the cathode 13. Usually about 2 mm separates the two electrode faces but the distance can range from about 1 mm to 10 mm.

As previously mentioned, the shaft 58 connects to the rear of the anode assembly and extends through the wall of the housing 12. Fluid leakage from the housing is contained by a flexible sleeve 64 (FIGS. 1 and 2). The shaft 58 serves to support and adjust the anode 14 to selected positions within the housing. Adjustment of anode position is effected by mounting the shaft in a mechanism 65 outside the housing which enables adjustment in an axial direction. For fine adjustments of the anode position, use is made of simple draw bolts 66.

As shown in FIG. 7, an electrical conductor 67 extends from the anode face 53 through the shaft 58 to the electrical power source. It is insulated except where it contacts the plates 53.

Metal-bearing electrolyte is introduced to the cell via a main feed line 90 and one or more of the valved branch lines 91, 92 and 93. Of these, conduit 91 connects to passage 61 in shaft 58 to supply electrolyte through the anode face into the housing. Conduit 92 connects through the wall directly into the interior of the housing. Conduit 93 connects to special conduit 75 on the scraper blade assembly for purposes to be more fully explained hereinafter.

Free gases, primarily oxygen, liberated in the cell, are withdrawn through the conduit 68 which connects to passage 63 in the shaft 58.

In the illustrated embodiment electrolyte will normally be supplied through both branches 91 and 92 to

keep the housing, including the inter-electrode space, full without excessive liquid movement transverse to the electrode faces. Thus, in the normal operation, fresh electrolyte enters through the anode surface and through the housing wall. Some electrolyte is withdrawn through the anode face with the gas and the balance is withdrawn through the flush conduit with the harvested metal.

To accommodate special conditions, such as the deleterious high acid that could occur in the recovery of zinc, a further inlet conduit 75 is provided to supply low-acid content feed electrolyte to the harvesting blade area to assist in flushing out the loosened metal while diluting the acid content of the spent electrolyte in which the metal is flushed from the cell.

A harvester is provided for continuously removing deposited metal from the cathode points. The harvester 72 (FIGS. 6-8) includes a blade 73 which is hooded, as hereinafter explained, and is fixed to a reciprocatable arm 74 which moves the blade and associated hood radially to-and-fro within a solid walled slot 76 formed in the anode face 53 (see FIG. 6). The blade, enlarged in FIG. 8, is much shorter than the slot 76. The blade extends toward the cathode face and terminates close to the cathode face so that as the cathode 13 rotates, the edge of the blade 73 scrapes the metal deposits from the cathode tips. At the same time, the arm 74 moves the blade gradually toward the center of the electrode. The result is that the blade cuts a spiral path. When the limit of travel is reached the blade returns rapidly to the starting position near the edge and the cycle is repeated. Spacers 73a are provided to separate the blade 73 from the bottom of the hood thereby permitting liquid and metal to flow around the blade to discharge via a tube 81 that connects from the interior of the hood to a remote location outside the cell, whereby the mixture of spent electrolyte and metal particles may be continuously flushed from the blade area thus removing metal from the cell as soon as it is scraped from the cathode. Flow through the discharge conduit is induced by the pressure of incoming fresh electrolyte entering through the supply conduits. The slurry of metal particles is conveniently conducted to a filter or other separator for final recovery of the metal.

Although other blade arrangements may be used to scrape metal from the cathode, it is important that only a relatively small percentage of clean cathode tips be exposed at any one time and that the major part of the total cathode area is normally covered by deposited metal. If too much cathode tip area is exposed without a corresponding reduction in total current then undesirably high voltages will occur at the cathode tips with the result that hydrogen will deposit on the cathode in preference to metal thus seriously interfering with the operation.

FIGS. 1 and 2 illustrate portions of the harvester mechanism exterior to the housing. A reciprocal hydraulic ram 78 is mounted to drive a carriage 79 mounted on tracks 80. The arm 74, which carries the blade on one end, has its other end connected to the carriage to reciprocate therewith. The arm enters the housing through a flexible sleeve 83. Controls (not shown), are provided to time the movement of the arm.

Electrolyte, such as an acid leach solution, is introduced via main conduit 90 and branches 91 and 92 into the housing thus feeding both through the anode face

and the housing wall to maintain the cell substantially filled with electrolyte.

The electrolyte flow rate, the applied voltage and the distance between the electrode faces are all adjusted to obtain the desired rate and quality of deposit. Typical current densities will range from about 0.5 to about 2.0 amperes per square cm (about 460 amperes/ft.<sup>2</sup> to about 1859 amperes/ft.<sup>2</sup>). As used herein, current densities are computed on total surface area of the cathode face - not just the cathode tips. The configuration of metal deposits on the cathode, except for some very soft deposits obtained at high current densities, is that shown in FIG. 5.

Simultaneously with the application of direct current, the cathode is rotated and the harvester blade actuated. The rate of cathode rotation and blade reciprocation are adjusted so that metal is scraped from the cathode tips fast enough to prevent bridging between adjacent deposits. Harvested metal and electrolyte are withdrawn from the cell via the conduit 81. Recovered metal particles are filtered and, if desired, compacted or ground to a high density powder.

During operation on a copper sulfate solution, free oxygen is liberated at the anode 14. A mixture of this oxygen and electrolyte is discharged through the porous anode face 53 thence through the conduit 68 to a separator and collector, not shown. The collected oxygen gas may be used as an oxidant in leaching or may be compressed for sale. Continuous removal of gas prevents polarization thus enabling electrolysis to proceed at minimum power consumption.

A test model constructed substantially as shown in the drawing was used for test work. In such model the cathode and anode were each 6 inches in diameter.

The cathode was formed from stainless steel wires, 0.075 to 0.125 mm in diameter  $\times$  2.5 mm length and were fixed in a flame sprayed ceramic matrix at an average spacing of 0.38 mm. Total cathode area, including the ceramic matrix, was 147 cm<sup>2</sup>.

The anode was constructed as described in connection with FIGS. 6 and 7. The anode face was formed from two layers of perforated titanium plate with 1.5 mm perforations. The plates were slightly spaced apart (1 mm) and the perforations were offset to create a tortuous path through the face. Twelve feed conduits 59 were provided in the anode face.

During tests, a purified electrolyte solution ranging from 10-35 g/l Cu and from 10-150 g/l H<sub>2</sub>SO<sub>4</sub> was supplied to the cell.

In a typical run, 2.82 volts was applied at 120 amperes total current (0.82 amp./cm<sup>2</sup>). Temperature was maintained at 86°C. The solution contained 130 g/l H<sub>2</sub>SO<sub>4</sub> and 15 g/l copper at CuSO<sub>4</sub>. Fresh solution was supplied to maintain these conditions and the test was run for 37 minutes during which time 79.6 grams of copper, at average particle size of 4-100 micron diameter, was collected. The copper exhibited a bulk density of 3.74 g/cc. Total power consumed was 0.208 Kwh and, under the test conditions, the power consumption rate was 2.68 Kwh/Kg Cu. Current efficiency was 90.8 percent.

These figures are contrasted with typical reported batch operations in conventional electrowinning in which current efficiencies as low as 72 percent and power consumption of 2.96 Kwh/Kg copper were attained at current density of 11 amperes/ft.<sup>2</sup>.

Under the foregoing conditions the new cell recovered copper at a rate of 1.81 lb. of copper per square foot/hour.

Whereas the invention has been described only with reference to permanent electrodes, it is not limited to such an arrangement. For instance, sacrificial anodes may be employed. Obviously the cell may be used in electro refining as well as electrowinning and it may be used to recover any metal susceptible to electrowinning.

Although the illustrated embodiment includes only a single anode and cathode, a single cell may employ a plurality of pairs of anodes and cathodes. The anode-cathode pairs may, in the same cell, be connected either in series or in parallel. The series connection is more attractive economically.

Although the cell may be formed in an open tank, the use of a completely closed cell enables operation at elevated temperatures without the release of free steam. This is advantageous because high temperature operation is desirable since it reduces electrolyte resistance and thus power consumption. Also, at a constant current density and electrolyte composition, a higher temperature will yield a metal product of higher bulk density and improved flow-ability.

If an open tank is used the inlet and outlet will be arranged to accommodate continuous feed and discharge while maintaining a constant volume of solution to keep the electrodes submerged to the desired degree.

Obviously the electrodes may vary in overall size; however, the dimensions and cross-sectional areas of the individual cathode conductors as well as the tip spacing should remain within the specified limits in order to achieve the desired results.

While the conductive cathode and anode surfaces are shown as being flat, it will be appreciated that embodiments utilizing other forms may be constructed. For instance, the conductive cathode surface may be cylindrical so long as it is smooth and presents a plurality of small conductors held in spaced-apart relationship by a matrix of non-conductive material. Similar comments apply to the anode.

As is the case in any electrical device, precaution must be taken to insure that the several elements are insulated as necessary to avoid shock hazard, shorting and the like. For instance, it will be necessary to insulate the scraper from the reciprocating shaft 74.

From the foregoing, it is evident that the present invention prevents novel ways and means for the continuous recovery of metal in electrolysis without interruption of the process.

I claim:

1. Apparatus for electrowinning of metal from a metal bearing electrolyte solution comprising a tank having an inlet and outlet and adapted to contain a substantially constant volume of electrolyte in continuous flow therethrough, an anode and a cathode mounted in said tank with conductive surfaces in functional relationship to each other, and said conductive surface of said cathode comprising a smooth surface formed from the free ends of a plurality of relatively small electrical conductors each of cross-sectional area in the range from  $0.0005\text{mm}^2$  to  $0.018\text{mm}^2$  and a matrix of non-conductive material holding said small conductors spaced-apart a distance of at least  $0.25\text{mm}$ .

2. Apparatus according to claim 1 in which said conductors are wires of diameter in the range from  $0.025$ – $0.15\text{ mm}$ .

3. Apparatus according to claim 1 in which said conductors are rectangular in cross section of dimension in the range  $0.025$ – $0.1\text{ mm}$  by  $0.5$ – $2.5\text{ mm}$ .

4. Apparatus for electrolytic recovery of metal from a metal bearing electrolyte solution comprising a tank having an inlet and an outlet for receiving and discharging electrolyte solution and arranged to maintain in said tank a quantity of solution having a predetermined upper level, at least one flat-faced anode and one flat-faced cathode in said tank said flat faces being respectively the conductive anode and the conductive cathode surfaces, said anode and cathode being arranged with their conductive surfaces in closely spaced face-to-face relationship and at an elevation such that at least a portion of both said conductive surfaces are below said predetermined upper level of solution, said conductive cathode surface comprising an exposed smooth surface formed from the free ends of a plurality of electrical conductors each of a cross-sectional area not exceeding  $0.25\text{mm}^2$  encapsulated in a matrix of non-conductive material to be held spaced apart at said surface a distance of at least  $0.25\text{mm}$ , means connecting said conductive anode and cathode surfaces to opposite poles of a source of direct current while said tank contains electrolyte solution thereby to effect deposition of small particles of metal on said free ends of said conductors on said conductive cathode surface, and means for dislodging said particles from said conductive cathode surface.

5. Apparatus according to claim 4 in which said means for dislodging metal from said conductive cathode surface comprises a scraper and means to effect relative movement between said cathode surface and said scraper.

6. Apparatus according to claim 5 in which said scraper is positioned between said conductive anode and cathode surfaces and product discharge conduit means are provided for withdrawing a mixture of solution and dislodged metal from adjacent said scraper.

7. Apparatus according to claim 6 with the addition of means for introducing a supplemental supply of electrolyte into the tank adjacent the inlet to said product discharge conduit means to provide at least part of the solution making up the mixture discharged from adjacent said scraper.

8. Apparatus according to claim 7 in which said conductive anode surface is porous, a plenum underlies said surface, and conduit means connect said plenum to a source of reduced pressure whereby to withdraw gaseous products through said anode surface.

9. Apparatus according to claim 4 in which said inlet includes means for introducing solution into the space between said conductive anode and cathode surfaces.

10. Apparatus according to claim 6 in which a slot with solid walls is formed in said conductive anode surface, said scraper is positioned in said slot and a reciprocatable means connected to said scraper is provided to effect back and forth movement thereof in said slot.

11. Apparatus according to claim 5 in which said means effecting relative movement between said cathode and said scraper comprises rotatably journalled shaft means connected to said cathode, and means outside said tank for rotatably driving said shaft and cathode.

12. Apparatus according to claim 6 in which said tank comprises a closed vessel and said inlet and outlet are arranged to maintain said tank substantially filled with solution.